

## UNITED STATES PATENT OFFICE

ALBERT L. CLAPP, OF DANVERS, MASSACHUSETTS

## MANUFACTURE OF WATERPROOF FIBROUS PRODUCTS

No Drawing.

Application filed September 27, 1928. Serial No. 308,880.

This invention relates to the manufacture of waterproof fibrous products, and has for its object to provide an economical method of uniformly waterproofing such products.

In manufacturing fibrous products, such as those made from cellulose pulp, it has heretofore sometimes been the custom to waterproof the pulp fibers in the beater engine by adding suitable sizing materials and precipitating such materials on the fibers before forming into the desired product and drying. When pulp so sized is used as a raw material in making moulded pulp articles, as for instance by introducing the pulp into foraminous moulds, then dewatering by forcing the pulp against the moulds by air, preferably in heated condition, under pressure, and finally removing the articles and drying, it has been found that considerable sizing material may be forced through the moulds along with the water of the pulp suspension, and is lost. In actual practice, it has been found uneconomical to incorporate more than about 5% sizing material in the pulp, since sizing material used in excess of this amount is apparently lost and tends to plug the moulds. This limited amount of sizing material, however, does not result in articles which are thoroughly waterproof, so that articles such as milk bottles require a special after-treatment with waterproof material, such as spraying with paraffin wax on the inside. Not only is such after-treatment expensive, but at best is a makeshift cure, since it is difficult to waterproof uniformly the inside of articles such as bottles.

I have discovered that a uniform suspension of pulp and molten thermoplastic waterproofing material, such as paraffin, may be prepared, if such molten material is agitated into a pulp suspension heated above the melting point of such material, and that such a heated mixed suspension may be made into fibrous products, for instance moulded fibrous articles, which are highly waterproof. The molten waterproofing material tends to coat the individual fibers, any excess remaining suspended in the form of discrete globules which permeate the fibrous product, filling the pores and interstices thereof. For instance, when the mixed suspension is introduced into foraminous moulds, the resulting article is highly waterproof, not only because the individual fibers are encased in waterproofing material but also because the discrete globules fill the pores and interstices of the article as the water in which they are suspended passes through the fibrous material and out of the mould. In order to avoid separation of the waterproofing material from the suspension, it is necessary that the suspension be maintained in agitated condition above the melting point of such material. Along with the waterproofing material, precipitable sizing material, such as 55 rosin size, may be added to the pulp, a suitable precipitant such as alum then being added to fix the sizing on the pulp fibers. The precipitate thus produced ensures a better and more uniform retention of molten waterproofing material on the fibers, as it tends to carry down and fix the suspended particles of molten material on the fibers. The process of the present invention further permits of the successful use of certain cellulose pulps which were heretofore found 60 unsatisfactory. Thus, in the moulding of articles, it has heretofore been necessary to use a free pulp, such as ground-wood pulp, since water may be removed quickly from 65 such pulp, and the moulded article is of sufficiently low water content to be handled. By moulding a heated pulp suspension as herein described, slowness is avoided even in 70 the case of pulps such as kraft and sulphite, so that articles of higher strength may be successfully moulded therefrom, owing to 75 the greater fiber length of such pulps. Articles such as milk bottles, when made as herein described, are practically sterile, bacteria and bacteria culture present in the pulp apparently having been destroyed by the elevated temperature treatment, which may 80 extend over a comparatively long period of time. This is an important feature of the 85 present invention, as heretofore pulp articles of the character described have been shown to contain a comparatively high bacteria content. Various thermoplastic waterproofing materials may be used in carrying out 90 95 100

the process of the present invention, materials such as paraffin, montan, carnauba, rosin, and asphalt having been found satisfactory when used independently or as mixtures.

5 The process of the present invention may best be appreciated by giving specific examples of procedure such as the following: One thousand pounds of wood pulp, made up 10 of, say, about 800 to 900 parts of blank news or ground-wood pulp and 100 to 200 parts of kraft pulp may be introduced into a beater engine, together with sufficient water to permit circulation and the proper beating out 15 or disintegration of the pulp, and the beater roll set in operation. The water used may be at elevated temperature, or else steam may be injected directly into the stock during 20 beating, the pulp thus being conditioned at a temperature of, say, 150° to 190° F., without being gelatinized or slowed down materially. Into the hot stock being beaten is then poured slowly 150 pounds of paraffin, 25 or mixture of 50 pounds of paraffin and 50 pounds of unsaponified rosin at 190° F., the molten thermoplastic material being of sufficiently low viscosity at this temperature to be uniformly disseminated throughout the 30 stock quite readily during the operation of the beater. The uniform suspension of pulp fiber and molten thermoplastic material, after beating for, say, about two to three hours at a temperature above the melting point of 35 the thermoplastic material, may then be sheeted or it may be introduced into moulds in such hot condition. The hot pulp suspension may be advantageously moulded into articles such as milk bottles, dishes, and toys, as by the so-called Drake process, the suspension 40 supply being maintained in hot condition while portions are being withdrawn and introduced into foraminous moulds faced with wire screening, heated air under pressure then being allowed to enter the moulds 45 to press the pulp against the screening and partially dry the articles, whereupon the articles are removed from the moulds and drying completed. It is found that the articles may be removed from the moulds with less 50 tendency to sticking and in much drier condition than was heretofore possible.

An important advantage of the process of the present invention is that it permits of the re-use of waste produced during manufacturing operations, as raw material. Thus, when articles such as milk bottles, waterproofed with paraffin, are being produced, imperfectly formed bottles or ones damaged by handling may be returned to the beater engine and treated along with the fresh raw material, the paraffined fibrous material being readily disintegrated into its constituent fibers at a temperature above the melting point of the paraffin.

55 Having thus described certain embodi-

ments of this invention, it should be evident to those skilled in the art that various changes and modifications might be made therein without departing from the spirit or scope of invention as defined by the appended claims.

70 I claim:

1. A process of making waterproof fibrous products having thermoplastic waterproofing material, which comprises mixing such material and a pulp suspension at a temperature above the melting point of such material, and forming the product from the suspension in such hot condition.

75 2. A process of making waterproof fibrous products having thermoplastic waterproofing material, which comprises heating a pulp suspension above the melting point of such material, mixing such material while in molten condition into the suspension, and forming the product from the suspension in such hot condition.

80 3. A process of making waterproof cellulose pulp products having thermoplastic waterproofing material, which comprises 85 beating a pulp suspension at a temperature above the melting point of such material, adding the material in molten condition to the suspension being beaten, and forming the product from the suspension in such hot condition.

90 4. A process of making waterproof fibrous products having thermoplastic waterproofing material, which comprises mixing such material and a pulp suspension at a temperature above the melting point of such material, adding precipitable sizing material, precipitating such material on the pulp fibers, and forming the product from the suspension in such hot condition.

95 100 5. A process of making waterproof pulp articles having thermoplastic waterproofing material, which comprises beating a pulp suspension at a temperature above the melting point of such material, adding the material while in molten condition to the suspension being beaten, moulding the suspension in such hot condition into articles, and drying the articles.

105 110 6. A process of making waterproof pulp articles having thermoplastic waterproofing material, which comprises beating a pulp suspension at a temperature above the melting point of such material, adding the material in molten condition to the suspension being beaten, moulding the suspension in such hot condition into articles, subjecting the wet moulded pulp to air pressure at elevated temperature to remove excess water, and drying.

115 120 125 7. A process which comprises heating a pulp suspension to a temperature of about 150° to 190° F., mixing molten thermoplastic material capable of being kept molten at such temperature with the pulp suspension, and

moulding the suspension in such hot condition into articles.

8. A process of making waterproof fibrous products, which comprises disintegrating fibrous stock associated with thermoplastic 5 waterproofing material above the melting point of such material, and forming the product from the resulting suspension in such hot condition.

10 In testimony whereof I have affixed my signature.

ALBERT L. CLAPP.

15

20

25

30

35

40

45

50

55

60

65